

# UNITED STATES PATENT OFFICE.

CHARLES S. DOLLEY AND ALBERT F. CRANK, OF PHILADELPHIA,  
PENNSYLVANIA.

## METHOD OF TAWING HIDES OR SKINS.

SPECIFICATION forming part of Letters Patent No. 629,124, dated July 18, 1899.

Application filed March 28, 1899. Serial No. 710,818. (No specimens.)

To all whom it may concern:

Be it known that we, CHARLES S. DOLLEY and ALBERT F. CRANK, citizens of the United States, residing at Philadelphia, in the county 5 of Philadelphia and State of Pennsylvania, have invented certain new and useful Improvements in Methods or Processes of Treating Hides, Skins, and Leather; and we do declare the following to be a full, clear, and 10 exact description of the invention, such as will enable others skilled in the art to which it appertains to make and use the same.

This invention relates to certain new and useful improvements in processes for treating 15 hides, skins, and leather; and the objects of the invention are to provide a process by means of which a superior leather can be produced either from raw hides or skins or from such hides or skins as have been previously 20 tawed or from such as have been partly but imperfectly tanned and which do not meet the various tests which are commonly employed to determine perfectly-tanned leather and which are therefore susceptible to im- 25 provement.

Certain varieties of skins (as is the case with E. I. kips and goatskins, basils, and white leather) are for convenience of shipment or for other reasons placed upon the market in 30 a tawed or an imperfectly-tanned condition. Such skins in many cases do not respond favorably to the usual tests for perfect leather, and hence require subsequent treatment.

Certain methods of tanning throw upon the 35 market a considerable amount of imperfect leather which is susceptible of improvement—as, for instance, that treated with cutch or terra-japonica, divi-divi, &c.—which if properly tanned would command higher prices.

40 It is one of the objects of the present invention to take such tawed and poorly-tanned leather and by proper treatment to convert the same into nearly perfect leather, thus greatly enhancing its value.

45 The invention has for a further object to fix in the skins or hides such substances—for example, extractives, coloring-matter, fillers, natural and artificial tannins, &c.—as may be employed with the purpose of feeding the 50 leather and of providing it with certain desired physical characters—such as plumpness,

weight, color, softness, impermeability to moisture, &c.

Our invention consists, essentially, of two steps, the first of which is concerned with the 53 introduction into the hide or skin of some material or materials which will render the skin sensitive to the fixing or tanning agent employed in the second step by overcoming the agglutinating action of the interfibrillar 60 ground substance (mucin, coriin, &c.) and effect a splitting up of the connective-tissue fiber bundles with an accompanying swelling and separation of the fibers and fibrils, pro- 65 ducing thereby a fulling or plumping effect, clearing the grain, and at the same time feed- 70 ing the leather—that is to say, impregnating the skin with materials the presence of which is desirable for the production of the physical qualities noted above. This first step has 75 the same purpose as that commonly attained by the employment of old and sour liquors and weak solutions of extractives and which precedes the actual tanning process.

The second step of the process consists in 75 treating the hide or skin to the action of formic aldehyde, ( $\text{CH}_2\text{O}_2$ ) a material possessing the property of fixing the connective-tissue fibers and fibrils in the swelled and plumped, tawed, or partially-tanned condition produced by the 80 first treatment and at the same time of fixing in, upon, or between the fibers and fibrils of the connective tissues materials which have been supplied by the first step of the process 85 to contribute special physical qualities—such as body, color, suppleness, weight, &c.—essen- 90 tial to a solid well-nourished leather. The use of the formic aldehyde in this second step is not a mere aggregation of elements or ma- 95 terials, as it is in its nature and effects en- tirely different from the materials employed in the first step and could not be substituted for them to produce the effects of the first step, while it possesses distinctive and positive characters by which it acts upon both the 95 skin and the materials with which it has been impregnated by the first step in a manner pec- 100uliar to itself, as will be hereinafter more fully set forth, and we use formic aldehyde in the second step of our process strictly as a tanning agent to render the skin non-putres- cible and insoluble.

In carrying out our invention we take advantage of the property possessed by various tawing and tanning agents—such as alum, salt, argol, eggs, flour, vegetable extractives, 5 gambier, and cutch, and the artificial and natural tannins used in making leather, many of which have none or only feeble tanning properties—of causing a swelling up or separation of the fibers and fibrils of the skin-connective tissue and the deposition in, upon, and between the same of materials which prevent them from again becoming agglutinated, thereby allowing the interlacing fibers to move readily upon each other and which at 15 the same time add material to the skin, which is of advantage in respect to weight, body, color, &c., whereby a plump, soft, pliable, tough, and elastic leather may be produced. Owing to the manifold qualities and varieties of leather required in the various industries it is impossible for us to specify any one 20 of the agents—such as alum, salt, eggs, flour extractives, reds, gambier, tannins, &c.—as being capable of meeting all requirements, 25 and in the first step of our process we hold ourselves free to use any or all materials which will produce the effect or effects desired—that is to say, the separation and swelling of the fibers and fibrils and the clearing and raising 30 of the grain, together with the plumping, filling, coloring, weighting, and rendering supple the skin—in short, its preparation for the subsequent fixing action of formic aldehyde as employed in our second step, an action in 35 some respects analogous to that ordinarily secured by means of those tannins which are capable of rendering gelatin insoluble, but in many respects peculiar to itself. The ultimate object of the invention in 40 using the materials designated in the first step of our process is to secure desirable states and qualities in the hides or skins treated, which may be fixed or supplemented therein by the action of formic aldehyde subsequently 45 applied in the second step, as hereinafter described. The following particular case will serve to illustrate the steps involved in our process: Commercial sheep or goat skins or hides, having 50 been previously prepared for treatment by softening, unhairing, or other necessary 55 and ordinary steps, usually referred to as "beam-house treatment," are placed in a drum or reel, in which they may be agitated by the revolving of the receptacle by paddles or by any other suitable means, the particular 60 method or mechanism employed constituting no part of the present invention. We hold ourselves free to employ any form of receptacle or method of agitation whatsoever. Together with the hides or skins in the receptacle is placed a solution of gambier extract 65 sufficiently diluted to present the extract to the entire mass of the skins, containing approximately four pounds of gambier to each one hundred pounds of wet hides or skins, the exact amount of gambier being based 70 on the weight of the skins or hides to be treated, also upon their acidity or alkalinity, according to well-known gambier-tanning processes. The skins or hides are then agitated in the gambier-bath until they are permeated through and through by the solution forming the bath, the time required depending somewhat upon the nature of the particular skins or hides, the size of the receptacle, the number or volume of skins, and the rapidity with which the receptacle is revolved or its contents agitated, factors which do not concern the principle involved in the process. 75 When the gambier has struck through or thoroughly permeated the skins, which may be ascertained by cutting into the thickest edge and examining the exposed interior, the skins are rinsed in clean water; but this washing or rinsing may, if preferred, be dispensed with and the second step proceeded with at once, and we do not wish to be held to washing the skins as a feature essential to our process.

We wish it clearly understood that the object of the first step of our process is, as has been previously stated, to bring the skins into a desired physical condition, characterized by such a separation and swelling of the tissue fibers and fibrils and such plumpness, weight, color, and suppleness as will, when fixed by the chemical action of formic aldehyde, constitute a superior leather of the particular character desired. Thus we are able to develop the desired physical characters by means of alum, salt, argol, eggs, flour, the tannins, gambier, and other vegetable extractives. In the first step, therefore, it is not so much a question of the materials employed, as there is a wide choice in this respect, but rather the securing of physical qualities in the skin, which we proceed to supplement, fix, and render permanent by the second step. The use of saline liquors serves to swell the tissues and fibers of the skin and to render it more readily affected by the tanning or fixing agent subsequently employed, while the vegetable extractives or their equivalents add color, weight, &c. The second step of our process consists in subjecting the skins or hides to the action of formic aldehyde, preferably in solution, although it may be employed in the state of gas, either in the same receptacle in which they were given the preliminary treatment or, if desired, in a special receptacle. The amount of the solution employed varies somewhat, but is based upon the weight of the skins or hides to be treated, and we have found in practice that three pounds of commercial forty-percent (40%) formic-aldehyde solution to each one hundred pounds of wet hides or skins is sufficient for ordinary sheep or goat skins. The amount of water with which the formic aldehyde is diluted is based upon the bulk of skins, being just sufficient to keep them well wetted and to present the formic aldehyde to the entire mass of the skins, but not so much as to dilute it.

not so much as to prevent the pounding action of the skins when revolving in the drum. The skins or hides are subjected to the action of formic aldehyde until permeated through 5 and through and until they respond to the usual tests for good leather. In the particular case which is cited herein as an illustration—namely, sheep or goat skins—we have found that the time required is approximately 10 three hours. The time, however, depends to a very considerable extent, as in the treatment by the first step of our process, upon the number of skins in the receptacle and the rate and mode of agitation to which they have 15 been subjected. It is advisable to maintain the bath in the second step at a temperature of not less than 80° Fahrenheit and not above 120° Fahrenheit in order to secure the greatest efficiency from the formic aldehyde, which 20 has greater penetration and less liability to polymerize than at low temperatures. After the skins are found to have been thoroughly fixed by the formic aldehyde they are washed and are then ready for the usual treatment 25 employed in finishing.

In case the formic aldehyde is employed in the state of a gas we prefer the following method: The skins having been brought to the desired state by the first step, as hereinbefore 30 described, an amount of commercial formic-aldehyde (forty-per-cent) solution, representing approximately three pounds to each one hundred pounds of wet hides or skins to be treated, is placed in a suitable generator, 35 a variety of which are upon the market, and the gas generated is allowed to pass by suitable connections into the chamber containing the skins. The temperature of this chamber is preferably maintained at from 110° to 120° 40 Fahrenheit, and the atmosphere of the chamber should also be kept moist, both of which conditions are readily secured by the admission from time to time of a small quantity of warm aqueous vapor by means of a suitable 45 steam connection. The chamber employed should be a closed one and no larger than necessary to allow the skins to be fully exposed to the action of the gas. If desired, the gas may be admitted to the drum in which the 50 preliminary treatment took place or into a similar drum and the skins agitated therein, or the skins may be stretched on suitable frames and inclosed within a stationary chamber, in either case being exposed to the action 55 of the gas until they respond to the usual tests for good leather—say for a period of six hours, the time depending, however, on the thickness and character of the skins under treatment.

60 The market supplies certain tawed or imperfectly-tanned skins and hides which have been already subjected to the action of salt and alum, flour, eggs, vegetable extractives, gambier, cutch, tannins, or other materials 65 and which do not constitute high-grade leather, but which are susceptible of improvement. The effects produced on these

skins are analogous to those produced by the first step of our process, and we find it both possible and advantageous to take such skins 70 and after softening them in water proceed to treat them as described in the example cited for treating raw skins, whereby we are able to secure the results of the first step with less time and material than would be required in 75 treating green or raw hides or skins, and in certain cases where the tawed or imperfectly-tanned skins or hides have the plumpness, color, weight, &c., desired and which we would have secured by means of our first step 80 we may proceed at once to the second step of the process, which consists, essentially, in the fixation of the natural or added constituents of the skin, substantially as described.

We have found by a large number of practical tests that the actual tanning effect of the natural tannins as introduced into the skin by the first step of our process may be greatly hastened and augmented by the employment of formic aldehyde in conjunction 90 therewith, as accomplished by the second step of our process. Thus with the pyrogal-lol tannins, a considerable proportion of which possesses little or no tanning power, a compound is formed whereby all the tannin is ren- 95 dered available, and consequently a greater action secured from a given amount of extract, a matter of importance in point of economy. Again, we find that by means of formic aldehyde used in conjunction with but 100 subsequent to the use of those natural (catechol) tannins, containing phlobophanes or “reds,” as introduced into the hides by the first step of our process, these substances, which in many instances are insoluble and 105 not directly available for tanning, can be fixed in the leather, and again with other (pyrogal-lol) tannins the deposit of “whites” or “bloom” is prevented, the ellagic acid or catechin being in some way altered and in- 110 dissolubly bound in combination with the skin substance, as are also certain extractives—e. g., gambier—by the action of the formic aldehyde upon the impregnated collagen of the skin, whereby an occlusion of the 115 introduced material is brought about; also, by its direct action upon the catechus themselves, whereby they are rendered insoluble and precipitated as a filling and coloring ma- 120 terial upon and between the fibers and fibrils of the skin-connective tissue, thus effecting what is technically known as “feeding” the leather. A special advantage afforded by our process is that it overcomes the obstacles 125 hitherto encountered in the use of materials like divi-divi, which add to the leather substances extremely susceptible to fermenta- 130 tion and which leads to loss of leather in damp weather. The superior bactericidal and anti-fermentative properties of formic aldehyde prevent this fermentation and the consequent softening of the leather. It also prevents molding during the drying of the unfinished leather.

Formic aldehyde has the property of fixing the collagen and other gelatinous constituents of the skin in the condition in which they are when subjected to its action, and we have found that it is highly advantageous in using formic aldehyde in the manufacture of leather to prepare the skins or hides by some preliminary treatment, as by our first step, whereby the fibers and fibrils of the connective tissue are properly separated and swelled or plumped, colored, or filled, as seems desirable in the particular case in hand, when they, together with the other gelatinous constituents of the skin, may be fixed in the particular state desired by the use of formic aldehyde, as has been previously described and which constitutes the second step of our process.

Our invention therefore proposes the application of formic aldehyde to hides and skins, the collagen of which is either not at all or but partially combined into insoluble compounds either, first, from a lack of suitable quality in the agents used in the preliminary treatment, such agents being, for example, salt, eggs, flour, alum, argol, vegetable extractives, gambier, cutch, and such other tannin-containing materials as possess little or no tannin properties, or, second, from lack of sufficient combination with an agent, such as oak or hemlock tannin, which is potentially capable of saturating the collagen and forming therewith an insoluble and imputrescible compound, but which in the skins we propose to treat has *de facto* not fully saturated the collagen. In other words, we propose to apply formic aldehyde to hides or skins containing a soluble collagen compound or unsaturated collagen. We therefore employ formic aldehyde to fix the collagen of the skins after the skins have been prepared by such processes as produce the qualities peculiar to ordinary salt-and-alum tawed skins, chamois leather, oil-tawed leather, wash-leather, Knapp's leather, &c., or the peculiar leather resulting from the employment of gambier and similar vegetable extracts, or where the fixation of the tissue constituents has been imperfectly accomplished by the ordinary tanning processes. The skins may be especially prepared or tawed skins. Chamois leather, &c., may be taken ready prepared and submitted to the fixing action of formic aldehyde.

Much of the leather commonly regarded as well tanned is open to great improvement, and our invention proposes the employment of the ordinary processes of tanning as our first step, or the taking of commercial leather already prepared by others and submitting it to the fixing and supplemental action of formic aldehyde as a second or final step in the production of perfectly-tanned leather.

Our invention therefore involves the use of formic aldehyde subsequent to the use of

tawing or tanning materials, and inasmuch as these materials give varying degrees of plumpness, weight, density, and color to hides and skins our invention necessarily involves the use of formic aldehyde in conjunction with all materials producing these effects in accordance with our process, as hereinbefore described.

We do not confine ourselves to the use of any one tawing or tanning, plumping, feeding, or coloring material in conjunction with formic aldehyde, as our process is not limited to the production of any one kind of leather, but is applicable to the production of either light or heavy leather, white or colored, as desired—in fact, to all varieties of leather—and its employment, as herein described, results in a very material saving in time, labor, and materials.

Having thus described our invention, what we claim to be new, and desire to secure by Letters Patent, is—

1. The process in the production of leather, which consists in subjecting skins or hides to tawing and tanning materials for the purpose of plumping, feeding, weighting or coloring them, and then submitting them to the fixing and tanning action of formic aldehyde.

2. The process in the production of leather, which consists in subjecting skins or hides to the action of tannin-containing extractives, whereby they are plumped, fed, weighted or colored, and then subjecting them to the fixing and tanning action of formic aldehyde.

3. The process in the production of leather, which consists in treating hides or skins with a tannin-containing extractive, capable of forming a combination with formic aldehyde, (e. g., gambier,) for the purpose of plumping, feeding, weighting or coloring them, and then subjecting the impregnated skins to the tanning and fixing action of formic aldehyde, whereby the material with which the skins have been fed, weighted and colored is fixed and occluded in the skin tissue, as the collagen of the skin is rendered insoluble and non-putrescible.

4. The process in the production of leather, which consists first in plumping, feeding, weighting, coloring or raising and clearing the grain of skins or hides by treating them in a bath of such agents, and to such steps as are commonly employed for this purpose, and subsequently fixing the skins or hides in the state thus secured and tanning the same by treating them in a bath of formic aldehyde.

In testimony whereof we affix our signatures in presence of two witnesses.

CHARLES S. DOLLEY.  
ALBERT F. CRANK.

Witnesses:

CHAS. O. MORTON,  
II. F. REARDON.

It is hereby certified that in Letters Patent No. 629,124, granted July 18, 1899, upon the application of Charles S. Dolley and Albert F. Crank, of Philadelphia, Pennsylvania, for an improvement in "Methods of Tawing Hides or Skins," errors appear in the printed specification requiring correction, as follows: Page 4, lines 2 and 13, the words "gelatinous" should read *gelatigenous*; and that the said Letters Patent should be read with these corrections therein that the same may conform to the record of the case in the Patent Office.

Signed, countersigned, and sealed this 29th day of August, A. D., 1899.

[SEAL.]

WEBSTER DAVIS,  
*Assistant Secretary of the Interior.*

Countersigned:

A. P. GREELEY,  
*Acting Commissioner of Patents.*